

W. E GREENAWALT.

## METALLURGICAL PROCESS.

APPLICATION FILED JUNE 10, 1918.

1,357,495.

Patented Nov. 2, 1920.

2 SHEETS—SHEET 1.



*WITNESSES*

WITNESSES  
S. Pearl Jacobs  
Cora M. Greenawalt

*INVENTOR*

INVENTOR.  
William C. Grammatt

FIG 1

W. E GREENAWALT.  
METALLURGICAL PROCESS.  
APPLICATION FILED JUNE 10, 1918.

1,357,495.

Patented Nov. 2, 1920.

2 SHEETS—SHEET 2.



**WITNESSES:**

J. Pearl Jacobs.  
Cora M. Greenawalt.

FIG 2

## INVENTOR

William E. Granville

# UNITED STATES PATENT OFFICE.

WILLIAM E. GREENAWALT, OF DENVER, COLORADO.

## METALLURGICAL PROCESS.

1,357,495.

Specification of Letters Patent. Patented Nov. 2, 1920.

Application filed June 10, 1918. Serial No. 239,255.

To all whom it may concern:

Be it known that I, WILLIAM E. GREENAWALT, a citizen of the United States, residing in the city and county of Denver and 5 State of Colorado, have invented certain new and useful Improvements in Metallurgical Processes, of which the following is a specification.

The invention has for its more immediate 10 object the rendering harmless, or mitigating the evils, in the electrolysis of impure electrolytes, especially electrolytes obtained from leaching ores and containing salts of the variable valent elements.

15 This process may be regarded as a continuation of my co-pending applications, Serial No. 15,583, and Serial No. 132,273, and, like those applications, will be described more particularly in reference to the 20 treatment of copper ores, although it is not intended to limit it to any particular use.

In the electrolysis of impure copper solutions, as for example those obtained from leaching copper ores with an acid sulfate 25 solution, there is always present iron sulfate, which injuriously affects the operation. Ferrous sulfate in the electrolyte is not particularly harmful, but the ferric sulfate is highly detrimental.

If a solution of copper sulfate, containing 30 ferrous sulfate, is electrolyzed, copper is deposited at the cathode while sulfuric acid and ferric sulfate are produced at the anode, as shown by the following equations:



40 The ferric sulfate, finding its way to the cathode, combines with the deposited copper, and is again reduced to the ferrous condition, thus:

45 3.  $\text{Cu} + \text{Fe}_2(\text{SO}_4)_3 = \text{CuSO}_4 + 2\text{FeSO}_4$ .  
The loss of efficiency due to this cause is more or less proportional to the amount of ferric sulfate in the electrolyte, and under certain conditions may be very large. In 50 aggravated cases the loss of efficiency may be so great that the copper is dissolved as rapidly as it is deposited.

If, however, the ferric sulfate can be reduced at the expense of a comparatively cheap reducing agent, such as hydrogen sulfid or copper sulfid, then acid is regenerated, and the iron in the electrolyte, being reduced to the ferrous condition, loses its ability to combine with the deposited copper, as shown by the equations:



In the treatment of copper ores by solvent processes there are produced rich and lean copper solutions. The rich copper solutions usually result from the application of the 70 standard solution, while the lean copper solutions usually result from the application of wash water to wash out the soluble values from the ore after the rich solutions have been withdrawn.

75 Usually, if the rich solutions are electrolyzed or not, the lean solutions are chemically precipitated and the precipitate so obtained usually plays no further part in the general metallurgical scheme. One of the 80 objects of this process is to use the sulfids precipitated from the lean, or from the foul solutions, to reduce, or eliminate, the difficulties in the electrolysis of the rich solutions, and have as an end product for both, 85 the pure electrolytic metal.

The process can best be described more in detail by referring to the accompanying drawings, in which Figure 1 is a diagrammatic longitudinal section, and Fig. 2, a 90 diagrammatic plan, of the general scheme and apparatus carrying it out. In the drawings, 1 is a leaching vat, or other suitable apparatus, for applying an acid solution to the ore to dissolve the copper. The rich copper solution flows into the storage tank 2, and forms the electrolyte. The lean copper solution, or washwater, flows into the pump 20, and is elevated through the pipe line 21 to the weak solution storage tank 22. From tank 22 the lean solution flows in a regulated stream into the precipitator 23, in which the solution is violently agitated, sprayed, or atomized, in the presence of hydrogen sulfid,

produced in the hydrogen sulfid generator 24. The copper is precipitated as the sulfid, with the simultaneous regeneration of acid, as set forth in the following equation:



The resulting sludge, consisting of the precipitated copper sulfid and regenerated weak acid solution, flows into the separator

- 10 25, in which the sulfid settles by gravity and is worked toward the central opening in the bottom and into the distributing pipe line 26 by the rotating mechanism within the tank, while the clear supernatant solution 15 flows into the oxidizer 28, through the pipe line 27. This oxidizer is preferably an electrolyzer in which the oxygen released by the electrolytic action, oxidizes any excess of hydrogen sulfid from the reducer, so that 20 the excess cannot precipitate copper in the ore as the more or less insoluble sulfid, and also to convert the ferrous salts into the ferric condition, which is desirable, since ferric salts act on both the sulfid and oxidized copper in the ore to bring it into solution. If oxidation is not desired, the solution flows through the by-pass 29. The washwater after having its copper precipitated and an equivalent of acid regenerated, 25 and preferably also electrolyzed to convert the ferrous salts into the ferric condition, is stored in tank 30 for re-use as an acid wash on the ore, as desired.

The electrolyte having the copper in solution and containing iron usually in both the ferric and ferrous condition, flows from the storage tank 2 in a regulated stream into the reducing unit 3, where the ferric salts are converted to the ferrous salts by means 35 of copper sulfid, then to the electrolyzers 4, then to the reducing unit 5, to the second series of electrolyzers 6, to the third reducing unit 7, to the third series of electrolyzers 8, and so on, until the electrolyte is sufficiently impoverished in copper and regenerated in acid. The reducing units consist of agitators, 3<sup>a</sup>, 5<sup>a</sup>, and 7<sup>a</sup>, of separators, 3<sup>b</sup>, 5<sup>b</sup>, and 7<sup>b</sup>, and of air-lifts, 3<sup>c</sup>, 5<sup>c</sup>, and 7<sup>c</sup>, or other device, for creating a return flow from 40 the bottom of the separator to the top of the agitator. The copper sulfid precipitate from the separator 25 is flowed in a regulated stream into the agitators 3<sup>a</sup>, 5<sup>a</sup>, and 7<sup>a</sup>, through the distributing pipe 26. The electrolyte and copper sulfid precipitate being 45 in this way brought into intimate contact, the ferric salts are quickly reduced to the ferrous condition. In order to make a clear separation of the precipitate and electrolyte after reduction, the overflowing reduced solution, still containing some copper sulfid in suspension, is passed to the thickeners or separators 3<sup>b</sup>, 5<sup>b</sup>, and 7<sup>b</sup>, where complete separation takes place; the clear overflow- 50 ing reduced solution going to the electro-

lyzers 4, 6, and 8, while the settled precipitate at the bottom of the separators is returned to the agitators, 3<sup>a</sup>, 5<sup>a</sup>, and 7<sup>a</sup>. In this way the copper sulfid precipitate is consumed and the electrolyte reduced and enriched in copper sulfate, as shown by equations 5 and 6. The electrolyzers 4, 6, and 8, are representative of a series of as many cells as desired.

The electrolyte on entering the cells is practically completely reduced. When electrolysis begins, copper is deposited at practically the theoretical rate, while acid is regenerated according to equation 1, and some of the ferrous salts converted to the ferric condition, according to equation 2. It is desirable to hold the ferric salts down to as low as 0.10% ferric iron; it should not, in any event, greatly exceed 0.25% ferric iron.

This may be conveniently done by having the cells in compound series and by regulating the rate of flow through the system. The ferric salts, as formed in alternate series of electrolyzers, is reduced in alternate reducers, and this is continued until the electrolyte is sufficiently impoverished in copper and regenerated in acid, when it flows into the pump 15, and through the pipe line 16 into the oxidizer and acid generator 17. This oxidizer is an electrolyzer in which the oxygen liberated by the electrolysis of the acid solution, oxidizes the ferrous iron to the ferric condition, so as to enable the solvent to act more energetically on the sulfids in the ore, which are unattacked by sulfuric acid. The solution may also be enriched in sulfuric acid by introducing sulfur dioxide, from the sulfur dioxide generator 18, into the oxidizer 17, where it is oxidized by the action of the electric current to sulfuric acid. If oxidation of the solution is not necessary or desired, it may be by-passed through the pipe line 31, into the storage tank 19. In either case the regenerated acid solution is stored in tank 19 to be applied to the ore in the leaching vat, as desired. The sulfuric acid acts on the oxids and carbonates, and the ferric iron on the sulfids. In this way a close extraction of the copper can be made—usually closer than by ordinary acid leaching.

The copper sulfid from the separator 25 may be directly distributed, through the pipe line 26, to the agitators 3<sup>a</sup>, 5<sup>a</sup>, and 7<sup>a</sup>. It is preferred, however, to introduce all the freshly precipitated copper sulfid into the first reducing agitator, 3<sup>a</sup>, and regulate the overflow in such a way that a considerable portion of the copper sulfid flows into the separator 3<sup>b</sup>, and then, as the settled sulfid is elevated by the air lift 3<sup>c</sup>, pass it on to the next reducing agitator 5<sup>a</sup>, where the cycle is repeated, and then on to the next reducing agitator, 7<sup>a</sup>, where the cycle is again repeated, and so on for the entire series of al-

ternate reducers and electrolyzers. When the impoverished sulfid sludge, containing also considerable quantities of sulfur as shown by equation 6, issues from the last 6 reducer, it is conducted to a filter 38, and the filtrate returned to the circuit through the pipe 43, while the sludge goes to the roasting furnace 39 to have the sulfur burned off, and the cupric sulfid partially converted into the 10 oxid, and partially into the cuprous sulfid by the elimination of one atom of sulfur. The cuprous sulfid is more effective in reducing the ferric salts than the cupric sulfid. The sulfid precipitate, treated to eliminate some 15 of its sulfur, is again put into the circuit 26 through the conveyer 40. The sulfur dioxid from the furnace may be conducted, through the pipe line 41 to the oxidizers, and acid generators, 28 and 17.

20 Instead of using air in the air lifts, 3<sup>e</sup>, 5<sup>e</sup>, and 7<sup>e</sup>, it might be desirable to introduce a gas into the air lift to act on the electrolyte. Either sulfur dioxid or hydrogen sulfid may be effectively introduced in this way. It 25 might be desirable to introduce sulfur dioxid in the electrolyte in the first reducer, 3<sup>a</sup>, and then maintain the ferric salts reduced with copper sulfid in the remaining reducers.

A partial reduction of the variable 30 salts may be made with sulfur dioxid, by diverting some of the gas from the sulfur dioxid generator 18, to the sulfur dioxid reducer 48, shown in Fig. 2.



Acid may be regenerated in this way from what would otherwise be a waste gas in many metallurgical works, while at the same time 40 reducing some of the ferric salts.

The process is applicable to chlorid as well as to sulfate solutions.

The reducing action of the precipitated 5 copper sulfid is positive in both hot and cold solutions. In hot solutions containing 3.5 grams ferric iron per liter, (0.35%), a 90% reduction can be made in five minutes at a temperature of 145 deg. F., with occasional stirring; under the same conditions, at 50 62 deg. F., 56% of the ferric iron can be reduced. Under the same conditions, in either hot or cold solutions, the ferric iron can be completely reduced in one minute by violently shaking in a bottle or violently agitating with air, when the amount of copper in suspension is equal to that in solution. As it is advisable to carry out the electrolytic 55 deposition at a temperature of about 125 deg. F., there should be no trouble in having a completely reduced electrolyte in the reducers, and effective depolarization in the cells, with considerably reduced power for the deposition.

55 I claim:

1. A metallurgical process which consists

in treating ores of copper with an acid solution to dissolve the copper, maintaining separate the resulting rich and lean copper solutions, electrolyzing the solutions rich in copper and containing salts of the variable 70 valent elements to deposit the copper whereby the salts of the variable valent elements are raised from a lower to a higher valency, treating the lean copper solutions to precipitate the metal as the sulfid, applying sulfur 75 dioxid to the rich solutions, and then maintaining the solution reduced with the copper sulfid obtained from the lean solutions.

2. A metallurgical process which consists in applying sulfur dioxid to a copper solution obtained from leaching ores and containing salts of the variable valent elements, electrolyzing the solution whereby the copper is deposited and the salts of the variable 80 valent elements raised from a lower to a 85 higher valency, maintaining the electrolyte reduced with copper sulfid until the electrolyte is sufficiently impoverished in copper and regenerated in the solvent, and then returning the electrolyte to the ore to dissolve more copper.

3. A process of electrolyzing a metal salt of a polybasic acid obtained from leaching ores and containing salts of the variable 90 valent elements which consists in alternately 95 electrolyzing and reducing the electrolyte by adding copper sulfid as a reducing agent in the first of the series of reducers and then carrying a portion of the reducing agent from the first to the last of the series of 100 reducers, and finally separating the impoverished reducing agent from the electrolyte impoverished in metal and returning the solution to the ore to pass through another 105 cycle.

4. A process of electrolyzing copper 110 sulfate solutions containing salts of iron which consists in alternately electrolyzing and reducing the electrolyte by means of copper sulfid as a reducing agent for the ferric salts formed by the electrolysis, adding the copper sulfid to the first of the series 115 of reducers and then carrying a portion of the copper sulfid from the first to the last of the series of reducers, and finally separating the impoverished copper sulfid from the electrolyte impoverished in copper and returning the electrolyte to the ore and treating the impoverished copper sulfid to reduce its sulfur content and again treating the 120 electrolyte therewith.

5. A process which consists in treating 125 ores of copper with an acid solution to dissolve the metal, maintaining separate the rich and the lean copper solutions, electrolyzing the solutions rich in copper and containing salts of the variable valent elements to deposit the copper, precipitating the copper from the lean solutions with a chemical precipitant, applying the chemical precipi- 130

tate to the electrolyte to reduce the higher valency salts formed by the electrolysis to a lower valency, and then before returning the electrolyte to the ore electrolyzing it under 5 different conditions to convert the lower valency salts to a higher valency.

6. A process which consists in treating ores of copper with an acid solution to dissolve the copper, maintaining separate the 10 rich and the lean resulting copper solutions, electrolyzing the rich copper solution containing salts of the variable valent elements to deposit the metal, precipitating the lean copper solutions with hydrogen sulfid, separating the sulfid precipitate from the weak acid solution, applying the copper sulfid to the rich solution to maintain the ferric salts reduced, and oxidizing the precipitated lean solutions by electrolysis and returning the 20 regenerated weak acid solutions to the ore.

7. In the electrolysis of a solution of a metal salt of a polybasic acid obtained from leaching ores and containing salts of the variable valent elements, the process which 25 consists in applying sulfurdioxid to the solution to reduce the salts of the variable valent elements from a higher to a lower valency in the first stages of the electrolysis, and then continuing the reduction of the higher 30 valency salts formed by the electrolysis by means of copper sulfid precipitate, and then when the solution is sufficiently impoverished in the metal being deposited and regenerated in acid returning the solution to 35 the ore.

8. In the electrolysis of a solution of a metal salt of a polybasic acid obtained from leaching ores and containing salts of the variable valent elements, the process which 40 consists in applying sulfur dioxid to the solution to reduce the salts of the variable valent elements from a higher to a lower valency in the first stages of electrolysis, and then continuing the reduction of the higher 45 valency salts formed by the electrolysis by means of concentrated copper sulfid, and then when the solution is sufficiently impoverished in the metal being deposited and regenerated in acid returning the solution to 50 the ore.

9. In the electrolysis of a solution of a metal salt of a polybasic acid obtained from leaching ores and containing salts of iron, the process which consists in electrolyzing 55 the rich metal solutions to deposit the metal and regenerate acid and ferric salts, precipitating the metal from the lean solutions as the sulfid, applying the metal sulfid precipitate to the electrolyte to reduce the ferric salts in the electrolyte and liberate sulfur from the precipitate, separating the residual precipitate from the electrolyte and reducing its sulfur content, and then again applying

ing the precipitate reduced in sulfur to the electrolyte. 65

10. In the electrolysis of a solution of a metal salt of a polybasic acid obtained from leaching ores and containing salts of iron, the process which consists in withdrawing the electrolyte from the electrolyzers into 70 pools at different points of the system, treating the withdrawn electrolyte at different points of the system with a solid reducing agent distinct from the ore by agitation, returning the reduced electrolyte to the electrolyzers, and finally when the electrolyte is 75 sufficiently impoverished in the metal being deposited and regenerated in acid returning the solution to the ore.

11. In the electrolysis of a solution of a 80 metal salt of a polybasic acid containing salts of iron, the process which consists in reducing the ferric iron formed by the electrolysis to the ferrous condition by applying a reducing agent to a series of pools of 85 the electrolyte, progressively advancing the electrolyte through a series of electrolyzers, and progressively advancing the electrolyte through a series of pools communicating with the electrolyzers and containing a reducing agent for the ferric salts. 90

12. In the electrolysis of a solution of a metal salt of a polybasic acid containing salts of iron, the process which consists in reducing the ferric iron formed by the electrolysis to the ferrous condition by applying a reducing agent to a series of pools of the electrolyte, progressively advancing the electrolyte through a series of electrolyzers, progressively advancing the electrolyte, 95 through a series of pools communicating with the electrolyzers and containing a reducing agent for the ferric salts, and progressively advancing the reducing agent through the series of pools of the electrolyte. 100

13. A metallurgical process which consists in treating ores of copper with an acid solution to dissolve the copper, electrolyzing the resulting solutions rich in copper and containing salts of iron to deposit the copper 110 with the simultaneous oxidation of the ferrous salts to the ferric condition, chemically precipitating the copper from the lean and foul solutions with hydrogen sulfid, separating the resulting copper sulfid precipitate 115 from the precipitated solution as a thickened sludge, and applying the copper sulfid precipitate in the form of a sludge to the rich copper solutions to reduce the ferric salts formed by the electrolysis to the ferrous 120 condition.

WILLIAM E. GREENAWALT.

Witnesses:

MARY H. WOOLSEY,  
IRMA GREENAWALT.